



2,796,655

## STRETCHABLE FABRIC AND METHOD OF MAKING SAME

Reinhold F. Stuewer, Scranton, Pa., assignor to Grove Silk Company, Scranton, Pa., a corporation of Pennsylvania

No Drawing. Application December 31, 1954.  
Serial No. 479,253

12 Claims. (Cl. 28—72)

This invention relates to a textile article having stretching properties superior to those exhibited by articles prepared from untreated yarn ends, and to the method of producing such article.

When synthetic fibers of the polyamide and polyester types, and in general the polymer synthetics which are formed by extruding a liquid through a nozzle, hardening and then stretching the filament, are subjected to setting operations at correlated temperature and time conditions, they thereby attain the capacity of returning toward the shape existent during the setting operation, in event of later mechanical twisting or untwisting, for example. Such yarns can be referred to as comprised of stretched microcrystalline polymers. When it is desired to increase the stretchability of a fabric made from multifil yarn, it has been proposed to set them in twisted form, so that the fabric is thus composed of individual knitted courses, wefts or warps, which have curls or twists in the filaments. In knitted fabrics there is a permissive stretchability in the loops formed in the knitting, and if a monofil or multifil yarn is made to have a

versely upon the setting temperature, other conditions being the same: for example the "dead" condition may occur at 14 turns untwisting (36 turns residual) after treatment at 170 degrees F., or at 12 turns untwisting (38 turns residual) at 200 degrees F.

The behavior of a synthetic yarn is largely determined by its history. Its disposition upon heating above room temperature, when without external stress, is to assume the

shape or relative position of the parts existent during the last prior setting operation: and it may develop internal stresses when detained against free return to such shape or relative position. In general, the effect of a setting operation can only be totally dissipated by a treatment which is more rigorous than the setting itself. For example, a yarn which has been twisted and set at 200 degrees F. in hot water undergoes a change of shape or relative positioning which is not completely eliminated by a later immersion in water at such temperature; and in practice some of the imposed twist will not be dissipated by treatment at 212 degrees F.

It has been found that a yarn having a pre-set behavior imposed at a relatively high temperature, which is then given a right-hand twist of 50 turns per inch and then set at a lower temperature while held in such twisted state, can then be brought to a non-lively or "dead" condition by partial untwisting by, say, 13 turns; and, furthermore, when the yarn in this non-lively condition is again subjected to a heat-treatment, it is activated and tends to untwist further by, say, 12 additional turns, thereupon exhibiting a liveliness condition corresponding to a left-hand twist of 12 turns. The amount of re-assumed liveliness can be determined by the conditions of the successive heat treatments.

It has thus been found feasible to produce stretchable

7

twist is right or left hand. When an original multifil yarn of 20 denier (7 filaments of about 3 denier each) is pre-set for 20 minutes in steam at 25 lbs. pressure, and then twisted 51 turns and twist-set at 200 degrees in humid air, the liveliness required removal of about 14 turns per inch: that is, more turns were removed than with a monofil of 20 denier. The product knitted satisfactorily as an essentially "dead" yarn. The fabric was treated in boiling water and developed liveliness in the yarn and a satisfactory stretch in the fabric.

Another example of multifil practice with 70 denier (34 filament) yarn, was to pre-set as before in steam at 25 lbs., then twist 65 turns per inch, and twist-set at 180-180. The yarn was essentially "dead" when 24 turns were removed, and was knitted. Upon treatment with 212 degrees steam, the yarn exhibited liveliness of 33 turns per inch through set-release.

A further example with 70 denier (34 filament) multifil yarn was to pre-set as before, then twist 103 turns per inch, and twist-set at 180-180. The yarn was essentially "dead" when 33 turns were removed, and was knitted. Upon treatment with 212 degrees steam, the yarn exhibited liveliness of 49 turns per inch, and the fabric had a crepe effect.

The amount of original twisting desirable for a given case depends upon the size of the filament, and the purpose of use. It must be sufficient to permit the untwisting, after setting, so that the yarn is non-lively at knitting, and to have a potential effect available upon set-release, to produce the desired liveliness of the yarn in the fabric. With filaments below 10 denier, e. g. at 1 or 2 denier, the twisting effect or liveliness in the fabric yarn may obviously be correspondingly higher: while at 20 and 40 denier, significant effects in wide gauge knit fabrics for example can be obtained with twists in the yarn of the fabric of less than 10 turns per inch, and even lower twists for greater diameters.

The removal of the liveliness from the twist-set yarn need not be accomplished upon the individual yarn. For example, two monofil or multifil yarns can be pre-set, twisted and twist-set, for example with both yarns having a left twist of 51 turns per inch. The two ends, without mechanical untwisting to remove the liveliness, can be plied together with, say, 8 turns of right-twist for 15 denier yarn: the bifilar product is then essentially "dead" and can be so knitted because the plying twist has removed the liveliness. The fabric, when knitted, can then be treated for set-release, whereupon the potential liveliness is developed in each yarn and gives the effect of a right-twist of, say, 25 or 26 turns. A like result can be attained with multifil yarns, e. g. two ends of 70 denier, 34 filament, yarns.

The temperature conditioning given to the twisted material can be referred to as "twist-setting": since its effect is to relieve some of the twisting stresses so that the yarn thus treated will not untwist completely when left free to adjust itself, but will have stored within it a condition of potential or residual untwisting ability although this is not exhibited by physical tendency to untwist further; and since it involves a second setting, subsequent to the historical treatment which pre-sets the filament or subsequent to the preferred pre-setting for stabilizing various yarns to a condition of like prior history of heat treatment.

The treatment of the yarn or fabric therefrom, by which such residual or potential twisting ability of the yarn is availed of for inducing liveliness therein, can be referred to as a "releasing" or "set-releasing" operation, since it causes residual or potential stress, resulting from the original twisting of the pre-set yarn, to become effective by release of the effect of the twist-setting.

Characteristic of this invention are the preparation of a yarn which can be knitted in essentially "dead" or non-lively condition but has within it the potential ability to attain a lively or twisting state thereafter even when present in a fabric, and the preparation of a fabric from

8

such yarn and the production in such fabric of the lively state of the yarn whereby the fabric contracts, and may exhibit a crepe effect, and assumes a correlated condition of stretchability.

5 The examples are illustrative; and the invention can obviously be practiced in many other ways in accordance with this disclosure and the scope of the claims.

I claim:

1. The method of making a stretchable fabric, which 10 comprises pre-setting yarn of stretched microcrystalline polymer at an elevated temperature below the adhesive temperature of the material and without significant tension thereon whereby to fix therein a condition toward which it returns during a later less rigorous heat treatment, twisting the yarn, twist-setting the yarn under conditions less rigorous than those of the pre-setting whereby a part of the strain produced in the yarn by the twisting is relieved and another part remains active therein, removing twist from the twist-set yarn so that it attains an essentially dead and non-lively condition with a potential twist therein, preparing a fabric from the yarn while in essentially dead condition, and thereafter subjecting the fabric to an elevated temperature under conditions effective for releasing a part of the potential twist 15 whereby the said yarn in the fabric becomes lively and the fabric contracts.

2. The method of making a stretchable fabric from stretched microcrystalline polyamide fiber yarn, which 20 comprises subjecting the yarn to pre-setting under elevated temperature conditions below the adhesion temperature of the material whereby to fix therein a condition toward which it returns during a later less rigorous heat treatment, twisting the yarn, subjecting the twisted yarn to twist-setting at an elevated temperature which is 25 not higher than 32 degrees F. below the pre-setting temperature whereby a part of the strain produced in the yarn by the twisting is relieved and another part remains active therein, removing twist from the twist-set yarn so that it attains an essentially dead and non-lively condition with a potential twist therein, preparing a fabric from the yarn while in essentially dead condition, and thereafter subjecting the fabric to an elevated temperature for releasing at least a part of the potential twist 30 under elevated temperature conditions less rigorous than those of the pre-setting whereby the said yarn in the fabric becomes lively and the fabric contracts.

3. The method of making a stretchable fabric, which 35 comprises pre-setting yarn of stretched microcrystalline polymer at an elevated temperature below the adhesive temperature of the material and without significant tension thereon and under humid conditions whereby to fix therein a condition toward which it returns during a later less rigorous heat treatment, twisting the yarn, heating the twisted yarn under humid conditions at a lesser temperature whereby a part of the strain produced 40 in the yarn by the twisting is relieved and another part remains active therein, removing twist from the yarn so that it attains an essentially dead and non-lively condition with a potential twist therein, preparing a fabric from the yarn while in such essentially dead condition, 45 and thereafter subjecting the fabric to a third heat treatment under humid conditions for releasing a part of the potential twist whereby the said yarn in the fabric becomes lively and the fabric contracts.

4. The method as in claim 3, in which the said third 50 heating is at a temperature less than the temperature of the pre-setting treatment.

5. The method as in claim 3, in which the said third heating is at a temperature greater than the temperature of the twist-setting treatment.

6. The method as in claim 3, in which the said third 55 heating is at a temperature not greater than the temperature of the twist-setting treatment.

7. The method of treating a yarn of stretched microcrystalline polymer, which comprises heating the same 60 under humid conditions to an elevated temperature below

the adhesive temperature of the material whereby to fix therein a condition toward which it returns during a less rigorous heat treatment, twisting the yarn, and heating the twisted yarn under humid conditions and at an elevated temperature below that of the pre-setting whereby a part of the strain produced in the yarn by the twisting is relieved and another part remains active therein, and removing twist from the twist-set yarn so that it attains an essentially dead and non-lively condition with a potential twist therein.

8. A fabric made in accordance with claim 1, and characterized in that the yarn thereof has residual potential twist therein.

9. A yarn made in accordance with the process of claim 7, and characterized in being in essentially dead and non-lively condition and having therein a potential twist which can be activated by subjection of the yarn to heating in a humid atmosphere.

10. The method of making a stretchable fabric, which comprises pre-setting at least two yarns of stretched micro-crystalline polymer at an elevated temperature below the adhesive temperature of the material and without significant tension thereon whereby to fix in each thereof a condition toward which the yarn returns during a later less rigorous heat treatment, twisting the yarns independently in the same direction, twist-setting the yarns under conditions less rigorous than those of the pre-settings whereby a part of the twist produced strain in the respective yarn is relieved and another part remains effective therein, plying the yarns with a plying twist in the opposite direction whereby the composite yarn attains an essentially dead and non-lively condition with a potential twist there-

in, preparing a fabric in a dead condition, and heating the elevated temperature of a major part of the composite yarn in the contracts.

11. The method of making a stretchable fabric independently pre-setting at least two yarns, the steps thereof, said in opposite directions, said two yarns in successive bands of the fabric being twisted together.

12. The method of making a stretchable fabric, the steps thereof being by knitting, and the knit goods.

#### References Cited

##### UNITED STATES PATENTS

|           |         |
|-----------|---------|
| 2,290,253 | Schnell |
| 2,564,245 | Billig  |
| 2,641,914 | Neumann |
| 2,662,558 | Mersch  |
| 2,772,191 | Burle   |
|           | FO      |
| 297,810   | Swit    |
|           | OT      |

1952, "American Hand Book of Textile Goods,"



June 25, 1957

J. W. SCHAPPEL ET AL  
MODIFIED REGENERATED CELLULOSE ARTICLES AND METHOD  
FOR MAKING THE SAME  
Filed Sept. 6, 1952

2,796,656



Fig. 1



Fig. 2